

Patented June 16, 1925.

1,541,819

# UNITED STATES PATENT OFFICE.

DANIEL DANA JACKSON AND ALLEN ROGERS, OF BROOKLYN, AND TE-PANG HOU, OF NEW YORK, N. Y.

## METHOD OF AND LIQUOR FOR PRODUCING TANNED LEATHER.

No Drawing.

Application filed September 2, 1921. Serial No. 498,049.

To all whom it may concern:

Be it known that we, DANIEL DANA JACKSON, ALLEN ROGERS, and TE-PANG HOU, said JACKSON and ROGERS being citizens of the

United States of America, and said HOU being a citizen of the Republic of China, said JACKSON and ROGERS residing in the borough of Brooklyn, city and State of New York, and said HOU residing in the borough of Manhattan, city and State of New York, have invented certain new and useful Improvements in Methods of and Liquor for Producing Tanned Leather, of which the following is a specification.

This invention relates to a tanned leather product, and to a method of tanning, and aims to provide improvements therein.

It has heretofore been proposed to tan hides and skins by the use of iron salts, but such methods as have heretofore been employed have not produced a satisfactory tanned product, the leather so produced being hard and stiff, and having a spotted appearance, shrinking and curling when dry, easily cracking on bending, deteriorating or rotting on keeping or storage, and being unfavorably affected by ordinary heat and light.

The present invention provides a method of tanning hides and skins, by the use of iron salts, whereby a good, useful leather may be obtained, which leather compares favorably, in its properties and appearance, with bark-tanned leather, or with chrome-tanned leather.

The invention further provides a leather, as the product of the present process, which is full and soft, which does not shrink or curl when dried, which, when dry, has a uniform color, free from dark, hard spots, which is not brittle, and does not crack on the grain, on sharp folding, which shows no deterioration on keeping or exposure to ordinary light or heat, which will not be de-tanned in contact with water, and which can be dyed, colored; or subjected to such dressing or currying operations as are, or may be, usually applied to leather tanned by other methods of tanning.

The invention further provides a method of producing a white tanned leather, by the use of iron salts, in conjunction with other salts, and a white leather product resulting from said method.

The invention also provides a method of

tanning with iron salts, capable of application in conjunction or combination with other kinds of tanning—such as vegetable tanning and oil tanning.

The invention further provides a novel tanning liquor.

According to the present invention, the hides or skins are treated in a tanning liquor containing ferric salts, and the ferric state is maintained throughout the period in which the hide is in the tanning liquor, by a suitable oxidizing agent, conveniently in 10 to 15% excess of the quantity for complete oxidation of the ferric salt, and by an after oxidation, as described hereinafter. According to our theory, the iron is combined with the hide in the ferric state, and the production of a satisfactory iron-tanned leather is due to the combination of the iron with the leather in a ferric state, and the maintenance of such conditions that the iron remains in such state until the tanning is completed.

The basicity of the ferric salt liquor is also to be considered, as it has been found to be important to start with such conditions of basicity that, when the hide or skin comes into contact with the liquor, no deposition of ferric oxid, as such, will take place on the hide, as is the case where a too basic liquor is used.

The general limits of basicity, we have found, on the basis of the ratio of the ferric iron to the mineral acid radical in the liquor, to lie between ratios of 5 equivalents of the acid radical to 6 equivalents of the ferric iron, and 3 equivalents of the acid radical to 4 equivalents of the ferric iron. In terms of laboratory analysis, this degree of basicity is conveniently taken as representing a mean of 30 c. c. of tenth normal sodium hydroxide for each c. c. of the iron liquor containing  $0.1gFe_2O_3$  to a c. c.

These limits of basicity of the tanning liquor are of importance, because, if the liquor employed is more acid than that indicated by the above mentioned limits, a permanent tanning action will not take place, whereas, if the liquor is less acid than indicated, a rapid precipitation of ferric oxid, on the hide or skin, will occur.

Heretofore, a too basic iron liquor has been employed, with the result that much light-yellow powder was precipitated in the liquor. A greater part of this precipitate

was deposited on the hide, imparting to it a light-yellow pigment color within a very short time (about 15-20 minutes in drum tanning). This mechanically deposited 5 powder has no tanning property, and, further, prevents the tanning salt from penetrating to the interior of the hide, which, hence, may remain untanned. Consequently, a hard, stiff, brittle, under-tanned leather 10 was produced.

A further quantity of the oxidizing agent is preferably added at or near the end of the tanning operation, conveniently an amount corresponding to the 10-15% excess 15 previously added. The oxidizing agent last added has the further advantage that the oxidation produced thereby serves to reduce the acidity produced during the tanning, and thereby conduces to the better fixation 20 of the iron in the hide.

After the tanning has been completed under the foregoing conditions, the hide or skin is treated to neutralize the acid in it. This may be carried out in the tanning bath, 25 or in a separate bath. It is preferable to effect the neutralization slowly and gradually, and it is further best to use a mild alkali, or, preferably, to use more than one alkali, starting with the milder alkali, such as 30 borax, sodium bicarbonate, or the like, afterwards making use of stronger alkalies.

After the hide or skin has been tanned, as described, and neutralized, it may be subjected to dressing or currying, or to combination tanning. 35

The dressing or currying may consist in the usual drying, rolling, stuffing, fat-liquoring, coloring, skiving, etc.

For oil combination tanning the iron tanned leather may be retanned in oil, as, for 40 example, cod liver oil, shark liver oil, or other (marine) drying fish oil. Such oil combination tanning is particularly suitable for the production of heavy leathers, such 45 as lace leathers, etc., where strength and tenacity are desired. Oil combination tanning may be effected by taking the iron tanned leather and drying it to a "sammied" state (or sammying it back from "crust"), 50 and drumming it for 4 to 6 hours in 20 to 30% of its weight of the fish oil, and afterwards hanging it out to dry.

To produce "stuffed" leather, the iron tanned leather may be treated with a mixture 55 of stearin, olein, and sulphonated cod liver oil. The leather may be drummed in this mixture, heated to about 140 degrees F., for about one-half hour. The stuffed leathers are suitable for harness, belting, etc., and the proportions of the oils may be varied, according to the particular use to which the leather is to be put.

For vegetable combination tanning, the 60 iron tanned leather may be retanned in a tannin-liquor obtained from hemlock, que-

bracho, chestnut, or other ordinary wood or bark used for the purpose. Such a liquor may be made by dissolving 10% of the solid powder (or 15% of the commercial extract), by weight, in enough water to give 15°-25° 70 Barkometer at a temperature of 90°-110° F. The iron tanned leather may be drummed in this liquor for about 2 hours, or the tanning may be carried out in a vat or paddle. Grey to black leathers are advantageously 75 produced by this vegetable combination tanning. Moreover, the vegetable combination tanning is of especial advantage in the tanning of skins and the lighter weight hides, as it gives a fuller and heavier leather; and, 80 at the same time, it may be utilized to effect a coloring of the leather. By using less astringent tannins, such as gambia, mimoso, sumac, pure oak, or spruce extract, a brownish-grey to greyish-black color is obtained, 85 depending on the kind of vegetable tannin used, the concentration of the liquor, and the duration of the tanning.

For dyeing the iron tanned leather, ordinary acid, basic, direct or alizarine dyes can 90 be used. For the case of basic dyes, and advisedly in the case of acid dyes, vegetable mordants, such as fustic, mimoso, gambia, or other vegetable tannins which do not produce a decided black with iron may be used, 95 and the colors applied as usual. No such mordants are required for direct or alizarine dyes. Black leather is preferably produced, as explained above, by combination vegetable tanning, and, where a deep black is desired, the combination tanned leather may 100 be topped with a black dye, as per example basic leather black. The temperature of the dye bath should preferably not exceed 140° F., between 130° and 140° F. being convenient 105 limits.

The following is a description of one particular example of the method of carrying out the iron tanning according to the present invention. 110

The tanning liquor may be prepared as follows: Ferrous sulphate crystals (copperas), of 12 to 14% of the weight of the drained hide or skin to be tanned, is placed in 1½ to 1¾ times its weight in water. It 115 is not necessary that the amount of water used be sufficient to dissolve completely all of the ferrous sulphate, inasmuch as the ferric sulphate that is formed when the ferrous sulphate is oxidized, as presently explained, has a higher solubility, mol for mol, than the ferrous sulphate. This condition as regards solubility may be utilized when a strong iron liquor is desired. 120

The ferrous salt is then oxidized to the 125 ferric state, by any suitable oxidizing agent. Chlorine, for example, may be used. Chlorine has an advantage as an oxidizing agent, in that it may be used in the cold, or at a slightly elevated temperature, between 70° 130

and 110° F., for example. It is also preferable to carry out the oxidation in a closed tank, and to admit the chlorine under a small pressure, (5 to 15 pounds gauge per square 5 inch, for example). The use of chlorine as an oxidizing agent has the further advantage that no acid requires to be added to the solution to effect the oxidation, and the solution consequently need not be made excessively acid. Moreover, the low temperature which may be employed with chlorine gives simplicity to the process, and the oxidized tanning liquor produced by its use 10 yields a very stable liquor for storage.

15 Sodium nitrate and sulphuric acid, or nitric acid and sulphuric acid, may also be used as oxidizing agents, in which case, however, a boiling temperature is required. After the oxidized iron salt solution has 20 been prepared, its basicity is regulated. For ordinary tanning purposes, from 50/100 to 65/100 pounds of soda ash per gallon of the liquor, prepared as described above, is added, and there is also preferably added from 1½ 25 to 2 pounds of salt per gallon of the liquor.

Instead of the above liquor, a tan liquor may also be prepared from a plain ferric salt, such as ferric chloride, ferric sulphate, etc. Ferric chloride yields a more stable 30 liquor than ferric sulphate, and the liquor has very little tendency to deposit hydrated ferric oxide in the basic solution. But it has perhaps a somewhat stronger oxidizing action than the ferric sulphate liquor.

35 The hides or skins, after being given the usual treatment prior to tanning, for example, soaking, unhairing, fleshing, washing, bating, pickling, as the case may be, are placed in the oxidized iron tanning liquor, prepared as above described. Approximately three gallons of the liquor, prepared according to the proportions set out above, is sufficient to tan 100 pounds of hide or skin. Conveniently, the liquor and hides are placed 40 in a drum, and the drum rotated to secure a thorough working of the liquor into the hide. It is preferable, in drum tanning, to dilute the tanning liquor, prepared as above described, to from 6 to 9 times its volume. It is also advisable, before starting the tanning operation, to rinse the drum with a 45 small quantity of bleaching powder.

50 The hide or skin is first worked in the drum for from one to one-and-a-half hours, at the end of which period a small quantity of an oxidizing agent, in solution, is introduced into the drum. The oxidizing agent may be conveniently bleaching powder, and the quantity of the bleaching powder used 55 in the solution which is introduced into the drum at this stage of the tanning operation may be from 1 to 2% of the weight of the hide or skin. If sodium bicromate be used 60 as the oxidizing agent, about ¼ to ¾% thereof, based on the weight of the hide, is

used. If other oxidizing agents be used, an amount equivalent to the sodium bicromate should be taken. The oxidizing agent which is used at this stage should be one which is able to effect oxidation with a low 70 acidity.

The working of the hide or skin in the drum is then continued for ten or fifteen minutes longer.

At the end of this time, the neutralization 75 of the acid in the hide or skin is begun. This is conveniently effected in the drum by the addition of an alkali having a mild action. For example, 4% of sodium carbonate, based on the weight of the hide, or 80 7% of sodium bicarbonate, or 12% of borax, dissolved in a small quantity of water, is preferably slowly, and in small portions at a time, introduced into the drum, conveniently while the drum is running, and 85 through the trunnion.

When several alkalies are used, it is preferable to use first the milder alkalies; in the case of the alkalies mentioned above, it is best to first introduce the borax or sodium 90 bicarbonate solution, and, afterwards, use the solution of sodium carbonate.

In place of sodium carbonate, a suspension 95 of calcium carbonate or magnesium carbonate, in somewhat less quantity, may be employed. These alkaline earth carbonates possess the advantage that an excess of them can be used without harm, and that this excess, when taken up by the leather, has a softening effect, and effectively prevents the 100 presence of sulphuric acid in the leather.

Owing to the strong coagulating effect which these alkaline earth carbonates have on the basic ferric salt, it is best to start with a weak alkali and introduce the alkaline 105 earth carbonates toward the end of the neutralization step.

Only from 70 to 80% of the theoretical quantity of the total alkali necessary to neutralize the acid in the liquor is needed, the 110 balance of the acid being permanently fixed in the hide or skin.

After the addition of the neutralizing agent or agents has been completed, the hide or skin is worked in the drum for about ten 115 minutes longer, and then conveniently rinsed in the drum. Thereafter, it may be drained and dried in the usual manner for dressing or finishing leather.

For tanning hides or skins, to produce a 120 white or light-colored leather, the iron tanning liquor, prepared as above described, together with a phosphate, may be used.

The hide or skin, after being tanned in the iron phosphate liquor, is treated with an alkali, to neutralize it; thereafter rinsed, and, if desired, given the usual finishing, dressing or currying treatment.

The following is a description of an example 125 of the method of carrying out the tan-

ning, with iron and phosphate salts, to produce white leather:

The hides or skins are first treated with the iron tanning liquor, prepared as above described, and containing the before described amount of alkali to provide the proper basicity, and also the amount of sodium chloride previously mentioned. The treatment is preferably carried out in a drum, in which the hides or skins are worked for about 1 to 1½ hours.

At the end of this time, there may be introduced a solution containing 4% of sodium pyrophosphate, with 2½% of sodium carbonate, the percentage being based on the weight of the hides or skins. The addition of this solution is preferably effected gradually. Instead of the pyrophosphate, any other soluble phosphate, or even a sparingly soluble phosphate, such as calcium phosphate, may be used. For example, tri-sodium phosphate may be used (6%), together with 1½% of sodium carbonate, or di-sodium phosphate may be used (5% together with 2½% of sodium carbonate). Instead of the sodium carbonate, an equivalent amount of any other alkali may be used, as, for example, sodium bicarbonate, borax, etc.

After the phosphate solution has been all added, the treatment or working of the hide or skin in the drum is continued for 10 to 15 minutes, after which it is rinsed, and is ready for the usual dressing or finishing treatment.

The relative proportions of the phosphate and alkali can be varied, according to the character of the leather to be obtained.

Another mode or example of carrying out the tanning, to produce white leather, is as follows:

The oxidized iron liquor, prepared as previously described, may have added to it a phosphate solution, as, for example, 4% sodium pyrophosphate, and the hides or skins treated in this, preferably in a drum, in which case the solution is diluted, as previously described. The duration of the treatment in the drum is from 3 to 5 hours.

The addition of the sodium phosphate solution serves to provide the proper basicity of the solution, so that the addition of alkali, for this purpose, is unnecessary.

Thereafter, the hides or skins are neutralized with 2½ to 4% of sodium carbonate,

or an equivalent amount of another alkali.

After rinsing, the hides or skins may be finished or dressed as usual.

While several particular modes of carrying out the process have been described, the invention is not to be understood as limited thereto, as the inventive ideas may be carried out in other particular modes.

What is claimed is:

1. A method of tanning, comprising oxidizing a ferrous salt solution to the ferric state, and adding an alkali to produce a basicity between ratios of 5 to 6 and 3 to 4 equivalents of the mineral acid radical to the ferric ion, and treating the pelt in said oxidized solution. 65

2. An iron tanning liquor, comprising a solution of an iron salt, completely in the "ic" state, and an oxidizing agent for preventing reduction of the iron, said solution 75 having a basicity between ratios of 5 to 6 and 3 to 4 equivalents of the acid radical to the ferric iron.

3. An iron tanning liquor, comprising a solution of an iron salt, completely in the 80 "ic" state, and an oxidizing agent for preventing reduction of the iron and a phosphate, said solution having a basicity between ratios of 5 to 6 and 3 to 4 equivalents of the acid radical to the ferric iron. 85

4. A method of tanning, comprising oxidizing a ferrous salt solution to the ferric state, and adding an alkali to produce a basicity between ratios of 5 to 6 and 3 to 4 equivalents of the mineral acid radical to the ferric ion, treating the pelt in said oxidized iron solution, and adding further quantities of the oxidizing agent towards the end of the treatment. 90

5. A method of tanning, comprising oxidizing a ferrous salt solution to the ferric state, and adding an alkali to produce a basicity between ratios of 5 to 6 and 3 to 4 equivalents of the acid radical to the ferric ion, treating the hides in said oxidized iron solution, adding further quantities of the oxidizing agent towards the end of the treatment, and neutralizing the acid in the pelt. 95

In witness whereof we have hereunto signed our names.

DANIEL DANA JACKSON.  
ALLEN ROGERS.  
TE-PANG HOU.